

Jan. 8, 1929.

1,698,166

F. W. MENZER

METHOD OF FORMING STENCILS

Filed March 23, 1927



Fig. 1.



Fig. 2.



Fig. 3.



Fig. 4.



Fig. 5.

WITNESS

M. Well

INVENTOR,  
Frederick W. Menzer,  
BY  
John Edward.  
ATTORNEY

Patented Jan. 8, 1929.

1,698,166

# UNITED STATES PATENT OFFICE.

FREDERICK W. MENZER, OF HAWTHORNE, NEW JERSEY.

## METHOD OF FORMING STENCILS.

Application filed March 23, 1927. Serial No. 177,563.

This invention relates to the manufacture of stencils and particularly stencils formed by coating bolting cloth or other more or less open mesh fabric (termed herein a foraminous screen) with some substance which is impervious to the color or the like used in printing with the stencil and of course except at the places where the figure openings are to be. Heretofore the practice has been to 5 coat the screen in the field, i. e., the whole area excepting the figure openings to be left. This was very tedious work where, as in stencils used for fabric printing and the like, the figures were complicated and close together, and it required considerable expenditure of time. Those who are skilled in the art know that the work could proceed much more quickly and be less tedious if any coating treatment which is to distinguish the figure areas from the field were applied in the 10 figure areas rather than in the field.

With this in view, and according to this invention, I coat a foraminous screen by placing thereon and one upon another two 15 substances so that one covers a greater area than the other and the area of the latter conforms to the stencil opening to be formed, the former substance being a liquid normally adapted to harden and the two substances 20 where they are in superposed relation to each other being reactive to form a coating portion less tenacious than the remainder of the coating, and thereupon work the coated screen until said coating portion is removed. In the 25 best practice of the invention the second named substance is also a liquid and I apply it first to the screen and it serves specifically to retard the hardening of the second substance as to the portion of the coating where they 30 are superposed.

In the accompanying drawing,

Fig. 1 shows a fragment of the screen with the figure outlines delineated thereon;

Fig. 2 is a similar view, showing the figure areas coated with the first substance;

Fig. 3 is a similar view, showing the entire area of the screen coated with the second substance except for a portion of the screen at one corner;

Fig. 4 shows the stencil completed i. e., the removing treatment having been effected so that the field remains coated but the screen is bare or denuded of coating within the figure openings; and

Fig. 5 is a fragmentary section on line

5-5 of Fig. 3, illustrating a detail of the method.

For the first coating substance I use fish glue, a solvent therefor (as acetic acid), a medium for retarding the drying of the glue (as glycerine) and fusel oil or alcohol or some other agent which will insure penetration of this substance, which it will be understood is in liquid form. The proportions may be as follows:

|                      |           |
|----------------------|-----------|
| Fish glue            | 2 oz.     |
| Acetic acid          | 4 oz.     |
| Glycerine            | 1 oz.     |
| Fusel oil or alcohol | 10 drops. |

70

As the second substance I may use Heinz's oil gold size, which is a liquid size used by painters and decorators for causing the adhesion of gold leaf to any surface and of course is normally adapted in time to harden 75 or set; this substance is composed of fat linseed oil, chrome yellow and japan drier, the term fat linseed oil meaning linseed oil that has been allowed to stand in an open vessel for such time that it becomes a very slow drying and pliable oil.

• First, according to the pattern selected, the figure is delineated on the screen 1, as at 2 in Fig. 1.

This having been done the first step, or 80 what I term the decorating step in the example of my method now being described, is to paint or otherwise coat so much of the screen area as is within each figure, as at 3 in Fig. 2, using the first substance.

Thereupon the entire area of the screen, including the portions covered by the first substance, is painted or otherwise coated with the second substance, as at 4 in Fig. 3; this may be conveniently done by spraying with 85 an air brush.

The coated screen is then left standing so that the hardening or setting of the second substance in the field can be completed preparatory to the step now to follow, which, if 100 the second substance is the one above specifically defined, will usually require about twelve hours. When this hardening ensues that portion of the coating which is within the figure area will be found capable of removal from the screen independently of the remainder of the coating, since the tenacity of the second substance within said area is depleted.

This removal, which results in the stencil 110

opening being formed, may be accomplished by working the coated screen in some such way as the following:

First the whole coated area of the screen 5 is rubbed, as with a cloth, and then it is washed with water. The rubbing removes the bulk of the coating within the figure area, and the washing removes any parts or particles of the coating that may then remain 10 on the otherwise bare screen so that the latter within the figure area is perfectly denuded.

My method results in the production of 15 stencils of the class described in which the figure openings, however complicated or close together, exist perfectly clear and clean-cut, and it wholly avoids the tedium and very much reduces the time at present required to produce such stencils.

20 I might first apply the second substance and then apply the other substance within the figure area excepting that the outline of the figure may be accomplished with greater nicety or sharpness if the first substance is 25 already present when the second substance is applied.

In producing figures with sharply defined 30 outlines I find it important to include in the first substance a penetrating agent. This causes said substance to pass clear through 35 and also straight through the fibrous structure of the screen, so that an area of absorption is in size and form the same on one side of the screen as on the other, or as indicated 40 diagrammatically at sectioned portion 3 in Fig. 5. In the absence of this the figure outline will be absent or at least less on what may be termed the reverse side of the screen 45 than on the obverse side (to which the substances are applied) and will frequently not be true to its intended form, so that when the second substance sets in the outlying area the effective resulting figure opening is not as intended.

45 Having thus fully described my invention, what I claim is:

1. The herein-described method of forming a stencil which consists in coating a foraminous screen by placing thereon and one upon

the other two substances so that one covers 50 a greater area than the other and the area of the latter conforms to the stencil opening to be formed, the former substance being a liquid normally adapted to harden and the two substances where they are in superposed 55 relation to each other being reactive to form a coating portion less tenacious than the remainder of the coating, and thereupon working the coated screen until said coating portion is removed therefrom.

2. The herein-described method of forming a stencil which consists in coating a foraminous screen by first placing thereon and so as to cover an area of prescribed form one substance and then placing upon the first substance and also upon the portion of the screen flanking said area a liquid substance normally adapted to harden, the first substance being active upon the portion of the second substance covering the same to retard the hardening thereof, allowing the second substance to harden as to the portion thereof not covering the first substance, and before the second substance has hardened as to the portion thereof covering the first substance working 75 the coated screen to remove so much of the coating as is within said area.

3. The herein-described method of forming a stencil which consists in coating a foraminous screen by first placing thereon and so as to cover an area of prescribed form a substance containing a liquid penetrating agent and then placing upon the first substance and also upon the portion of the screen flanking said area a liquid substance normally 85 adapted to harden, the first substance being active upon the portion of the second substance covering the same to retard the hardening thereof, allowing the second substance to harden as to the portion thereof not covering the first substance, and before the second substance has hardened as to the portion thereof covering the first substance working 90 the coated screen to remove so much of the coating as is within said area.

95 In testimony whereof I affix my signature.

FREDERICK W. MENZER.